

Feb. 16, 1971

YUTAKA NEICHI ET AL

3,563,898

Mg-Mn-Al FERRITE BODY FOR MICROWAVE APPLICATION

Filed Aug. 22, 1967



Fig. 1



Fig. 2



Fig. 3.

yutaka Neichi

Misora Sugimura and  
Eiichi Hirota, Inventors

B. y. Wenderoth, Lind & Poole, Atteg

## 1

3,563,898

### Mg-Mn-Al FERRITE BODY FOR MICROWAVE APPLICATION

Yutaka Neichi, Hirakata-shi, Minoru Sugimura, Neyagawa-shi, and Eiichi Hirota, Sakai-shi, Japan, assignors to Matsushita Electric Industrial Co., Ltd., Osaka, Japan

Filed Aug. 22, 1967, Ser. No. 662,520  
Int. Cl. C04b 35/26

U.S. Cl. 252—62.58

2 Claims

#### ABSTRACT OF THE DISCLOSURE

A ferrite body useful in making e.g. microwave circuit elements and having narrow  $\Delta H$  characteristics, relatively high Curie temperature, low saturation magnetization, small coercive force and good squareness ratio is constituted by a Mg-Mn-Al ferrite composition with a porosity less than 2% and an average grain size of 0.5 to  $20\mu$  or 100 to  $500\mu$ . Optimal compositions comprise MgO 45 to 50 mol percent, Fe<sub>2</sub>O<sub>3</sub> 35 to 45 mol percent, Al<sub>2</sub>O<sub>3</sub> 5 to 15 mol percent and MnO 0.1 to 7.0 mol percent. Improved  $\Delta H$  is achieved by the additional presence of 0.1 to 5 wt. percent of Y<sub>2</sub>O<sub>3</sub>, ZrO<sub>2</sub> or Bi<sub>2</sub>O<sub>3</sub> or 0.1 to 5 wt. percent of additional MgO. A "site ratio" of Mg ions from 0.5 to 0.2 is desirable.

This invention relates to a microwave circuit element and more particularly to ferrite bodies adapted for microwave applications, and especially to ferrite compositions consisting of Mg-Mn-Al ferrites, and also to a method for making such ferrite bodies.

Recent electronic engineering has required a ferrite composition suitable for use in microwave applications such as in circulators, insulators and gyrators. Particularly a development in a non-reciprocal circuit in the V.H.F. or U.H.F. region requires a special ferrite with high resistivity, low saturation magnetization value, and high Curie temperature. Such applications require especially a ferrite body having a narrow ferromagnetic resonance line width  $\Delta H$ , a small coercive force and a good squareness ratio in the hysteresis loop.

Accordingly, it is a principal object of this invention to provide a sintered polycrystalline ferrite body having a narrow  $\Delta H$  characteristics for use in a non-reciprocal circuit in the U.H.F. or V.H.F. region.

Another object of the invention is to provide a square-loop ferrite composition with a relatively high Curie temperature, a low value of saturation magnetization and a small coercive force.

A further object of the invention is to provide a method for making a ferrite body having narrow  $\Delta H$  characteristics accompanied with a relatively high Curie temperature, a low saturation magnetization, a small coercive force and a good squareness ratio.

These and other objects of the invention will be apparent upon consideration of the following detailed description taken together with the accompanying drawings wherein:

FIG. 1 is a perspective view of an illustrative circulator comprising two ferrite bodies and a strip conductor;

## 2

FIG. 2 is a graph illustrating the line width versus the porosity of said sintered ferrite;

FIG. 3 is a graph illustrating the line width versus the average grain size of said ferrite in accordance with the invention.

5 Before proceeding with the detailed description of the microwave circuit element contemplated by the invention, an example of the construction thereof will be described with reference to FIG. 1 of the drawing wherein reference character 10 designates, as a whole, a microwave circuit element having, as active component, preferably disc-shaped bodies 1 of ferrite body according to the present invention.

Said bodies 1 are attached together through strip conductor 2 and are magnetized with an external magnetic field perpendicular to the surface of said ferrite bodies 1.

The ferromagnetic resonance line width  $\Delta H$  is defined as the distance  $\Delta H$  on the field scale at a constant frequency between the sides of the ferromagnetic resonance absorption curve at mid-height, as expressed in the literature, for example, "Ferromagnetic Resonance," chap. I, Sec. 10, p. 66, edited by S. V. Vonsovskii, Pergamon Press, 1966. The line width  $\Delta H$  is measured by a cavity resonator method at a frequency of about 9600 mc.

20 According to the present invention a Mg-Mn-Al ferrite body provided with a porosity less than 2% and an average grain size less than  $30\mu$  or higher than  $100\mu$  produces a narrow ferromagnetic resonance line width,  $\Delta H$ .

25 A superior  $\Delta H$  can be achieved by employing a Mg-Mn-Al ferrite body having a porosity less than 2% and an average grain size of 0.5 to  $20\mu$  or 100 to  $500\mu$  in accordance with this invention.

30 Moreover, according to the present invention the  $\Delta H$  of said Mg-Mn-Al ferrite having a porosity less than 2% and an average grain size less than  $30\mu$  or higher than  $100\mu$  can be further lowered by air-quenching the sintered body from a temperature higher than 1200° C.

35 The average grain size is determined by calculating the number of grains in a given area of a microscopic photograph in a given magnification in association with a method defined at pages 1690 to 1693 of the 1955 Book of ASTM, i.e. E89-52. The porosity of the ferrite is defined by the following formula:

$$45 P = \frac{(D_x - D)}{D_x} \times 100(\%)$$

where  $D_x$  is X-ray density and  $D$  is bulk density.

50 A Mg-Mn-Al ferrite is known to be of a mixed spinel structure in which Mg ions occupy partly the A-sites and partly the B-sites of the structure. The present ferrites have the following formula:

$$55 vMgO \cdot wMnO \cdot xMn_2O_3 \cdot yAl_2O_3 \cdot zFe_2O_3$$

Where  $v+w=1$ ,  $x+y+z=1$  and  $0.7 \leq z < 1.0$ ,  
 $0.002 \leq y \leq 0.3$

59  $0.9 \leq v \leq 1.0$  and  $0 \leq w+2x \leq 0.2$ . The cation distribution in the ferrite is

$$(Mg_{v\pm}Mn_{w+2x}Fe_{2z})[Mg_{v(1-\pm)}Fe_{2z(1-\pm)}Al_{2y}]O_4$$

60 where ( ) and [ ] denote an A-site and B-site of the spinel lattice, respectively. The site ratio of Mg ions at

the A-sites to those at the B-sites, namely  $\xi/(1-\xi)$ , can be controlled by a heat-treatment. That is, the ratio of a given composition is determined by a heating temperature and a cooling rate from said heating temperature to room temperature (about 15 to 30° C.).

According to the present invention the  $\Delta H$  of

### Mg-Mn-Al

ferrite depends greatly on said site ratio. An optimal site ratio of Mg ions is from 0.2 to 0.5 in accordance with the present invention.

Said site ratio of a given composition varies with the heating temperature and is frozen at room temperature by rapid quenching. A desired site ratio can be obtained by controlling the final heating temperature and the cooling rate in association with the weight of heated samples. A conventional method for obtaining a desired site ratio is to air-quench the ferrite body from the final heating temperature to room temperature. A more precise method is to reheat the furnace-cooled body having a specified porosity and average grain size at a temperature at which a desired site ratio is achieved and to air-quench individually the reheated body to room temperature. The site ratio frozen at room temperature can be determined by a saturation magnetization method disclosed by E. W. Gorter, Philips Res. Rep. 9 (1954) 295-365, 403-443, "Saturation magnetization and crystal chemistry of ferromagnetic oxide."

A ferrite body having a porosity less than 2% and an average grain size less than 30 $\mu$  can be prepared by employing a hot-press technique. A mixture of a desired composition is charged to a silicon-carbide die which can be supplied with a compacting pressure through punches during heating by using a pressing machine. Said die is preferably lined with a material inert to said ferrite composition. Said mixture is initially heated to a sintering temperature of 1100° C. to 1450° C. without any pressure at a heating rate of 100° C./hr. to 1000° C./hr. by any available and suitable heating method. Said mixture is maintained at said sintering temperature for 30 minutes to 6 hours while being pressed at a pressure of 50 to 5000 kg./cm.<sup>2</sup>. After pressing, the hot-pressed body is air-quenched to room temperature of about 15 to 30° C.

A ferrite body having a porosity less than 2% and an average grain size higher than 100 $\mu$  can be achieved by employing a hot-press technique which differs slightly from that suitable for making a ferrite body having a porosity less than 2% and an average grain size lower than 30 $\mu$  as mentioned above. A mixture of a desired composition is charged to a refractory die which can be supplied with a compacting pressure through punches during heating by using a pressing machine. Said refractory die is made of any suitable refractory material such as silicon carbide, silicon nitride or graphite and optimally is lined with a material inert to said ferrite composition. Said mixture is initially heated to a sintering temperature of 1100° C. to 1400° C., without applying any pressure, at a heating rate of 100° C./hr. to 1000° C./hr. and is maintained at said sintering temperature for 30 minutes to 10 hours while being pressed at a pressure of 50 to 500 kg./cm.<sup>2</sup>. After pressing, the hot-pressed body is heated to a temperature higher by at least 50° C. than said first temperature and is maintained at that temperature for 30 to 180 minutes without pressing. Subsequently, the heated body is air-quenched to room temperature of about 15 to 30° C.

Referring to FIG. 2, curve A illustrates the relation of  $\Delta H$  to the porosity of an Mg-Mn-Al ferrite body of an average grain size of 30 $\mu$  and furnace-cooled from 1300° C. Said Mg-Mn-Al ferrite consists of 47.5 mol percent of MgO, 2.5 mol percent of MnO, 2.0 mol percent of Mn<sub>2</sub>O<sub>3</sub>, 7 mol percent Al<sub>2</sub>O<sub>3</sub> and 41 mol percent of Fe<sub>2</sub>O<sub>3</sub>. It will be clear from the curve A that the  $\Delta H$  increases with an increase in the porosity and is low at a porosity less than 2%.

Curve B in FIG. 2 illustrates the relation of the  $\Delta H$  to the porosity of an Mg-Mn-Al ferrite of an average grain size of 30 $\mu$  and air-quenched from 1300° C. The composition of the Mg-Mn-Al ferrite is the same as that of the ferrite body of the curve A. It will be clear from the curve B that the air-quenching process remarkably improves the  $\Delta H$ .

Curve C of FIG. 2 illustrates the relation of the  $\Delta H$  to the porosity of an Mg-Mn-Al ferrite body of an average grain size less than 10 $\mu$  and air-quenched from a temperature of 1300° C. The composition of said Mg-Mn-Al ferrite is the same as those of the ferrite bodies of the curves A and B. It is readily understood that the  $\Delta H$  can be further lowered by making an average grain size less than 10 $\mu$  in addition to air-quenching and by making the porosity less than 2%.

The effect of the average grain size on the  $\Delta H$  of an Mg-Mn-Al ferrite having a porosity of about 2% is shown more clearly by the curve of FIG. 3. Said

### Mg-Mn-Al

ferrite body consists of the same composition as that of the Mg-Mn-Al ferrite body of FIG. 2 and is air-quenched from a temperature of 1300° C. The  $\Delta H$  increases with an increase in the average grain size up to about 70 $\mu$  and decreases with an increase in the average size as shown in FIG. 3. It will be clear that a low  $\Delta H$  can be obtained with an Mg-Mn-Al ferrite body having an average grain size excluding a value of about 30 to 100 $\mu$ .

The optimal base composition of said Mg-Mn-Al ferrite is listed in Table I:

TABLE I

|                                      | Preforable<br>mol<br>percent | Optimal<br>mol<br>percent |
|--------------------------------------|------------------------------|---------------------------|
| Ingredients:                         |                              |                           |
| MgO-----                             | 45-50                        | 45-50                     |
| Fe <sub>2</sub> O <sub>3</sub> ----- | 35-49.9                      | 35-45                     |
| Al <sub>2</sub> O <sub>3</sub> ----- | 0.1-15                       | 5-15                      |
| MnO-----                             | 0-10                         | 0.1-7.0                   |

A further improvement in the  $\Delta H$  can be achieved by adding 0.1 to 5.0 weight percent of Y<sub>2</sub>O<sub>3</sub> or ZrO<sub>2</sub> or MgO to said base composition listed in Table 1 in association with the specified porosity, average grain size and site ratio.

Furthermore, according to the present invention the composition of Table 1 with or without additives of Y<sub>2</sub>O<sub>3</sub> or ZrO<sub>2</sub> can be provided with a higher Curie temperature suitable for use in a non-reciprocal circuit element by incorporating therein 0.1 to 5.0 weight percent of Bi<sub>2</sub>O<sub>3</sub>.

Following are examples of the presently-preferred illustrative embodiments of the invention.

### EXAMPLE 1

A mixture consisting of the following composition of Table 2.

TABLE 2

|                                      | Mol percent |
|--------------------------------------|-------------|
| Fe <sub>2</sub> O <sub>3</sub> ----- | 41          |
| Al <sub>2</sub> O <sub>3</sub> ----- | 7           |
| MgO -----                            | 47.5        |
| MnO <sub>2</sub> -----               | 4.5         |

is calcined at a temperature ranging between 800° C. and 1200° C. for 3 hours in air and cold-pressed into a disc form. The pressed disc body is fired at a temperature of 1350° to 1400° C. for a time period of 2 to 20 hours in air and is furnace-cooled or air-quenched to room temperature of 15° to 30° C. The cooled disc is then lapped at the surfaces into a form 0.1 mm. thick and 1.5 mm. diameter. The resultant disc is examined with respect to average grain size, porosity, the site ratio of Mg ions and the  $\Delta H$ , the results being indicated in Table 3.

TABLE 3

|            | Firing<br>Sintered             |                         |                   | Average<br>grain<br>size, $\mu$ | Porosity,<br>percent | Site<br>ratio | $\Delta H$ ,<br>oe. |
|------------|--------------------------------|-------------------------|-------------------|---------------------------------|----------------------|---------------|---------------------|
|            | Calced<br>temp., $^{\circ}$ C. | Temp.,<br>$^{\circ}$ C. | Periods,<br>hours |                                 |                      |               |                     |
| Sample No. |                                |                         |                   |                                 |                      |               |                     |
| 1          | 1,200                          | 1,350                   | 5                 | Furnace-cooled                  | 15                   | 4.1           | 0.2                 |
| 2          | 1,000                          | 1,350                   | 5                 | do                              | 15                   | 3.0           | 0.2                 |
| 3          | 900                            | 1,400                   | 10                | do                              | 30                   | 2.0           | 0.2                 |
| 4          | 800                            | 1,400                   | 15                | do                              | 30                   | 1.2           | 0.2                 |
| 5          | 1,200                          | 1,350                   | 2                 | Air-quenched                    | <10                  | 5.0           | 0.42                |
| 6          | 1,200                          | 1,350                   | 5                 | do                              | 15                   | 3.8           | 0.42                |
| 7          | 1,000                          | 1,350                   | 5                 | do                              | 15                   | 3.0           | 0.42                |
| 8          | 1,000                          | 1,400                   | 10                | do                              | 20                   | 2.5           | 0.44                |
| 9          | 900                            | 1,400                   | 10                | do                              | 25                   | 2.0           | 0.44                |
| 10         | 800                            | 1,400                   | 15                | do                              | 30                   | 1.2           | 0.44                |
| 11         | 800                            | 1,40                    | 200               | do                              | 30                   | 1.0           | 0.44                |

## EXAMPLE 2

30 grams of a calcined mixture having a composition of Table 2 is hot-pressed, using a SiC die provided with SiC punches. The die containing the calcined mixture is heated to a temperature of 1300° to 1450° C. without applying pressure and then is kept at said temperature for a time period of 1 to 6 hours while applying a pressure of 50 to 500 kg./cm.<sup>2</sup>. After hot pressing, the die containing the hot-pressed body is air-quenched to room temperature of 15 to 30° C. The hot-pressed body is cut and lapped into a disc of 0.1 mm. thick and 1.5 mm. diameter. The  $\Delta H$  of the resultant disc is measured at 9600 m.c.; the results are listed in Table 4 as a function of the grain size, porosity, and the site ratio of Mg ions.

TABLE 4

| Sample No.: | Hot pressing                       |                |                                   | Average<br>grain<br>size, $\mu$ | Porosity,<br>percent | Site<br>ratio | $\Delta H$ ,<br>oe. |
|-------------|------------------------------------|----------------|-----------------------------------|---------------------------------|----------------------|---------------|---------------------|
|             | Temper-<br>ature,<br>$^{\circ}$ C. | Time,<br>hours | Pressure,<br>kg./cm. <sup>2</sup> |                                 |                      |               |                     |
| 12          | 1,350                              | 3              | 150                               | <10                             | 1.3                  | 0.41          | 60                  |
| 13          | 1,400                              | 3              | 150                               | <10                             | 1.0                  | 0.43          | 50                  |
| 14          | 1,450                              | 6              | 300                               | <10                             | 0.5                  | 0.44          | 40                  |

The magnetic and electrical properties of the ferrite are as follows: a saturation magnetization  $4\pi Ms \sim 1800$  e.m.u./cc., Curie temperature  $Tc \sim 210$ ° C., a coercive force for  $Hc < 0.8$  oe., a squareness ratio  $Br/Bm > 0.8$  and a resistivity  $\rho > 10^6$  ohm-cm.

## EXAMPLE 3

A calcined mixture having a composition according to Table 2 is hot-pressed after the manner described in Example 2. The die containing the calcined mixture is heated up to 1350° C. without applying pressure and then is kept at the said temperature for a time period of 5 hours while being pressed at a pressure of 300 kg./cm.<sup>2</sup>. After pressing, the hot-pressed body is heated to 1450° C. and maintained at this temperature for 2 hours without pressing, and thereafter is air-quenched to room temperature. The average grain size of the hot-pressed ferrite is 100 $\mu$  and the  $\Delta H$  is 65 oe. Other properties are similar to those described in Example 2.

## EXAMPLE 4

A mixture of the composition set forth in Table 2 is calcined at 1000° C. for 1 hours in air and then cold-pressed into disc form. The pressed body is fired at 1400° C. for 20 hours in air. The fired body is air-quenched from the firing temperature of 1400° C. or is cooled gradually to various temperatures of 1300°, 1200° and 1000° C. so as to be air-quenched from the various temperatures to room temperature of 15° to 30° C. Before being air-quenched, the disc is kept at various temperatures for 5 hours so as to be in an equilibrium state with respect to the site ratio of Mg ions at the respective temperatures. The  $\Delta H$  of the resultant disc is measured after the manner of the foregoing examples, and the results are listed in Table 5 as a function of Curie temperature, saturation magnetization and the site ratio of Mg ions. The resultant disc has a porosity of about 1.2% and an average grain size of 30 $\mu$  regardless of the quenching temperature.

TABLE 5

| 20 | Quenching<br>temp.,<br>$^{\circ}$ C. | $\Delta H$ , oe. | Curie<br>temp.,<br>$^{\circ}$ C. | $O_{\text{sat}}$ ,<br>e.m.u./g. | Site<br>Ratio <sup>1</sup> | Sample No.: |    |
|----|--------------------------------------|------------------|----------------------------------|---------------------------------|----------------------------|-------------|----|
|    |                                      |                  |                                  |                                 |                            | 15          | 16 |
| 25 | 1,400                                | 65               | 213                              | 53.5                            | 0.435                      |             |    |
|    | 1,300                                | 70               | 221                              | 49.5                            | 0.408                      |             |    |
|    | 1,200                                | 76               | 232                              | 39.0                            | 0.338                      |             |    |
|    | 1,000                                | 102              | 235                              | 35.0                            | 0.266                      |             |    |
|    | 26                                   | 115              | 239                              | 28.0                            | 0.188                      |             |    |

<sup>1</sup>  $(Mg^{3+}_{x}Fe^{3+}_{0.47-x}Mn^{2+}_{0.05}Mn^{3+}_{0.08})[Mg^{2+}_{0.95-x}Fe^{3+}_{0.77+x}Al^{3+}_{0.22}]O_4$ ; here ( ) denotes A and B-site in spinel type lattice, respectively.

Site ratio=Number of Mg ions at A site/number of Mg ions at B site.

<sup>2</sup> Furnace-cooled.

30

## EXAMPLE 5

40 The composition according to Table 2 has incorporated therein 0.1 to 10.0 weight percent of additive  $Y_2O_3$ ,  $ZrO_2$  or  $Bi_2O_3$ . The mixture is treated after the manner described in Example 1 so as to be formed into a disc. The fired disc is air-quenched from 1400° C. The  $\Delta H$ ,  $Tc$  and  $4\pi Ms$  of the resultant disc is measured and listed in Table 45 6. The site ratio of the resultant disc is about 0.44 and does not vary with addition of various weight percents of the additive.

TABLE 6

| 50 | Additive    | Curie<br>temperature,<br>$^{\circ}$ C. |                  | $4\pi Ms$ ,<br>e.m.u./cc. |
|----|-------------|----------------------------------------|------------------|---------------------------|
|    |             | Material<br>Weight,<br>percent         | $\Delta H$ , oe. |                           |
| 55 | Sample No.: |                                        |                  |                           |
|    | 20          | 0.1                                    | 50               | 200                       |
|    | 21          | 1.0                                    | 40               | 195                       |
|    | 22          | 5.0                                    | 55               | 103                       |
|    | 23          | 10.0                                   | 105              | 180                       |
|    | 24          | 0.1                                    | 55               | 200                       |
|    | 25          | 1.0                                    | 40               | 200                       |
|    | 26          | 5.0                                    | 50               | 1,900                     |
|    | 27          | 10.0                                   | 95               | 205                       |
|    | 28          | 1.0                                    | 55               | 1,750                     |
|    | 29          | 1.0                                    | 60               | 221                       |
|    | 30          | 5.0                                    | 70               | 253                       |
|    | 31          | 10.0                                   | 85               | 1,600                     |

## EXAMPLE 6

65 The composition of Table 2 has incorporate therein the additives listed in Table 7. The mixture is treated after the manner of Example 6. The  $\Delta H$ , Curie temperature and  $4\pi Ms$  of resultant disc are measured and the results are listed in Table 7.

TABLE 7

| Additives                                           | $\Delta H$ , oe. | Curie<br>temp.,<br>$^{\circ}$ C. | $4\pi Ms$ |
|-----------------------------------------------------|------------------|----------------------------------|-----------|
| 1.0 wt. percent $Y_2O_3$ +5.0 wt. percent $Bi_2O_3$ | 65               | 255                              | 1,750     |
| 1.0 wt. percent $ZrO_2$ +5.0 wt. percent $Bi_2O_3$  | 70               | 260                              | 1,700     |

70

75

## SCHEDULE OF ABBREVIATIONS AND SYMBOLS

## Abbreviation

| symbol:        | Meaning                                               |
|----------------|-------------------------------------------------------|
| D              | Bulk density.                                         |
| D <sub>x</sub> | X-ray density.                                        |
| P              | Porosity.                                             |
| ΔH             | Ferromagnetic resonance line width.                   |
| T <sub>c</sub> | Curie temperature.                                    |
| H <sub>c</sub> | Coercive force.                                       |
| B <sub>r</sub> | Residual magnetic inductance.                         |
| B <sub>m</sub> | Maximum magnetic inductance.                          |
| ρ              | Electrical resistivity.                               |
| σ <sub>s</sub> | Saturation magnetic moment.                           |
| M <sub>s</sub> | Saturation magnetization.                             |
| V.H.F.         | Very high frequency ranging from 30 mc. to 300 mc.    |
| U.H.F.         | Ultra high frequency ranging from 300 mc. to 3000 mc. |
| E.m.u.         | Electro-magnetic unit.                                |
| A- and B-      |                                                       |
| site           | Cation lattice site of spinel lattice.                |

## What is claimed is:

1. A microwave circuit element comprising a Mg-Mn-Al ferrite body having a porosity less than 2%, a site ratio of Mg ions from 0.2 to 0.5, and an average

grain size ranging from 0.5 to 500 $\mu$  excluding 30 to 100 $\mu$ , said ferrite body having a basic composition comprising 45 to 50 mol percent of magnesium oxide, 35 to 50 mol percent of ferric oxides, 5 to 15 mol percent of aluminum oxide and 0 to 5 mol percent of manganese oxide, wherein said basic composition additionally contains 0.1 to 5 wt. percent of at least one member selected from the group consisting of Y<sub>2</sub>O<sub>3</sub>, ZrO<sub>2</sub> and Bi<sub>2</sub>O<sub>3</sub>.

5 2. A microwave circuit element according to claim 1, 10 wherein said basic composition additionally contains 0.1 to 5 wt. percent of MgO.

## References Cited

## UNITED STATES PATENTS

|    |           |         |              |           |
|----|-----------|---------|--------------|-----------|
| 15 | 3,002,929 | 10/1961 | Van Vitert   | 252—62.58 |
|    | 3,034,986 | 5/1962  | Baird et al. | 252—62.64 |
|    | 3,023,165 | 2/1962  | Van Vitert   | 252—62.58 |
|    | 3,189,550 | 6/1962  | Malinofsky   | 252—62.62 |

20 TOBIAS E. LEVOW, Primary Examiner

R. D. EDMONDS, Assistant Examiner

U.S. CL. X.R.

25 252—62.64